

July 23, 1929.

G. H. WILLIS

1,721,982

RUBBER HEEL

Filed July 2, 1928

*Fig. 1*



*Fig. 2*



*Fig. 3*



Inventor  
Glenn H. Willis  
By Robert McPheron  
Atty.

Patented July 23, 1929.

1,721,982

# UNITED STATES PATENT OFFICE.

GLENN H. WILLIS, OF AKRON, OHIO, ASSIGNOR TO JOHN L. SNYDER, OF AKRON, OHIO.

## RUBBER HEEL.

Application filed July 2, 1928. Serial No. 289,733.

This invention relates to laminated rubber material or articles such as rubber shoe treads and particularly heels, of the type employing a non-metallic attaching layer.

5 My object in connection with heels and the like is to dispense with the use of embedded metallic washers now commonly employed for the purpose of retaining the nail heads, thus reducing the labor cost, and at the same 10 time to avoid the objections to other substitutes which have been proposed such as wood, fiberized rubber, or rubberized cloth, which detract from the flexibility and resiliency of the heel or exhibit other disadvantages such 15 as relatively-poor adhesion between the cushion body and the attaching layer.

In the preferred mode of practicing the invention I employ a heel having the usual concave seating face in which is inserted a flexible, resilient inlay of rubber composition including an intermixture of elongated or 20 filiform organic reinforcing material capable of imparting to the inlay a leathery firmness without greatly suppressing its rubbery 25 characteristics. This inlay or attaching layer is joined to the rubber cushion body with an inseparable vulcanized bond and serves as an effective means of retaining the nail heads, preventing spreading of the heel and obtaining 30 a tight seating at the edges.

Of the accompanying drawings,

Fig. 1 is a top plan view of a rubber heel embodying my invention.

Fig. 2 is a perspective view of the attaching plug or layer.

Fig. 3 is a sectional view of a portion of a heel mold containing the heels; which are shown in transverse section.

In the drawings, 10 is the resilient heel body composed of a suitable rubber compound such as good reclaimed rubber, with or without new rubber, and containing the usual pigments, sulphur for vulcanization and accelerator.

45 The attaching layer is a shallow inlay or plug 11 composed of rubber compound of about the same quality as the body compound, or it may be a cheaper quality, together with an intermixture of organic reinforcing material capable of imparting to the vulcanized compound a firmness resembling that of oak-tanned sole leather, but without entirely suppressing its rubbery characteristics—including resiliency and capability of forming an inseparable vulcanized bond with the body 50 rubber. The reinforcing material is indi-

cated at 12, homogeneously distributed throughout the rubber compound used in the plug 11.

The plug or layer 11 is located in the mold 60 13 with the aid of guide pins 14 on the lower mold plate, so that it will retain its proper position in the seating face of the heel under the pressure of the molding operation. The body rubber 10 being placed over said plug 65 11, the mold is then closed and the heels vulcanized as to both members thereof in a single heat, the plug requiring no preliminary semi-cure.

The molding pressure will cause the edges 70 of the plug 11 to flow outwardly somewhat beyond the pins 14 while the rubber is in a plastic state, but the plug is embraced or surrounded in the seating face, preferably on all sides as shown in Fig. 1, by the body rubber 10, said plug being thus inlaid or embedded flush in the seating portion or face.

The seating face of the heel being shaped in concave form in the usual manner, as indicated in Fig. 3, the attaching layer 11 acts 80 like a stiff spring when the heel is nailed down to its seat on the shoe, and the softer edges of the body rubber coat therewith to insure a tight seating all around.

The guide pins are located outside of the 85 usual nailing zone or area which surrounds the central area of the attaching face so as to leave said nailing area imperforate, this being a construction which I prefer because it avoids having to place the nails accurately 90 at predetermined points in said nailing zone. Any other desired means for holding the inlay in place during the molding operation may be substituted for the pins 14.

95 As a material 12 for reinforcing the rubber compound in the attaching layer 11 I have successfully employed animal hair of various kinds, including hog hair, oriental (human) hair, goat hair and cattle hair; all of which are relatively-stiff and tough as 100 compared with soft animal or vegetable fibers such as cotton, wool, etc.; and of these, the one I consider the best on account of its cheapness and general suitability for the purpose is common hog hair. This is used in the proportion of approximately 30% on the total weight of the compound in the layer 11, but this proportion is subject to some variation. In this connection, animal hair is 105 sharply distinguished from vegetable fibers like cotton and from asbestos on account of its coarseness and marked springiness or re-

siliency in the rubber compound, together with the fact that it imparts the necessary stiffness to the attaching layer without impairing the capacity of said layer to form an integral vulcanized union or an autogenous welded joint with the plain rubber compound of the heel body.

The rubber stock in the layer 11, for mixing purposes, should be made rather soft or 10 sappy as by the use of about 5 to 6% of a flux or softener such as cottonseed oil, palm oil or a suitable mixture of vegetable and mineral oils, in order to facilitate the distribution of the hair throughout said stock.

15 Milling is preferably performed on even-speed rolls having an open setting to avoid a bank, and the hair is fed to the space between the rolls into the plastic sheet which follows one of said rolls, the opening being 20 increased as the volume builds up. It results from this method of incorporating the hair that the latter retains substantially the effective length in the compound which it had before being introduced thereto. That is, if hog 25 hairs of the ordinary length of from  $\frac{1}{2}$  inch to 3 inches and averaging about  $1\frac{1}{2}$  inches are used, it will be found that this process of milling breaks only the longer ones, leaving the shorter ones unbroken and the average 30 hair length after milling the compound will be nearly 1 inch. A hair only  $\frac{1}{2}$  inch long is so firmly anchored in the rubber that it cannot be pulled out without breaking.

When a homogeneous mixture has been obtained, the compound is run into a sheet of the desired thickness and flat blanks or plugs 35 11 of the shape shown in Fig. 12 are died out of said sheet. These plugs are then assembled in the mold 13 with the body rubber in 40 any suitable manner and the heels vulcanized as already described.

A heel constructed as above set forth can be made at a reduced labor cost as compared with the common type having embedded me-

tallic washers, and the results are superior, 45 not only in comparison with such type but also as compared with heels employing other substitutes for washers which have heretofore been proposed. The nails readily penetrate the layer 11 but their heads are effectively retained thereby, an inseparable bond with the body rubber is obtained, the stiffness of the layer 11 prevents the attached heel from spreading and contributes to a tight seating 50 at the edge, and the heel as a whole, including the attaching layer, is both flexible and 55 resilient.

I claim:

1. A composite, vulcanized-rubber shoe 60 tread which is flexible and resilient throughout, said tread comprising a rubber cushion wearing body, and an attaching layer of leathery firmness integrally vulcanized to said cushion body and formed of rubber intermixed with relatively-long animal hair, 65 said layer being adapted to retain nail heads and resist the lateral spreading tendency of the cushion body.

2. A composite, vulcanized-rubber heel 70 comprising a rubber cushion body, and a flexible, resilient, attaching layer integrally united with and inlaid in the seating face of said body, said layer being composed of rubber compound containing a minor proportion of animal hair having substantially the stiffness of hog hair.

3. A composite, vulcanized-rubber heel 75 comprising a rubber cushion body, and a flexible, resilient, attaching layer integrally united with and inlaid in the seating face of 80 said body, said layer being composed of rubber compound containing a minor proportion of animal hair having substantially the stiffness of hog hair and of an average length of not less than one-half inch.

In witness whereof I have hereunto set my hand this 29th day of June, 1928.

GLENN H. WILLIS.